# EUROPEAN PATENT SPECIFICATION

(11) **EP 0 494 860 B1**
(45) Date of publication and mention of the grant of the patent: **27.12.1995**
(21) Application number: 90905073.4
(22) Date of filing: 20.09.1989
(51) Int. Cl.: C10L 1/12, C10L 1/32, C10L 9/10

(54) **METHOD FOR REDUCING SOX EMISSIONS DURING THE COMBUSTION OF SULFUR-CONTAINING COMBUSTIBLE COMPOSITIONS**
VERFAHREN ZUR ERMÄSSIGUNG DES AUSSTOSSES VON SCHWEFELOXYDEN WÄHREND DER VERBRENNUNG VON SCHWEFEL ENTHALTENDEN BRENNSTOFFEN
PROCEDE DE REDUCTION DES DEGAGEMENTS D'OXYDES DE SOUFRE PENDANT LA COMBUSTION DES COMPOSITIONS COMBUSTIBLES A TENEUR EN SOUFRE

(43) Date of publication of application: 22.07.1992
(73) Proprietor: Intevep SA, Caracas 1010 A (VE)
(72) Inventor: HAYES, Michael, E., Fernandina Beach, FL 32034 (US); HREBENAR, Kevin, R., Jacksonville, FL 32211 (US); MINOR, Jennifer, L., Lenexa, Kansas 66215 (US); WOODWORTH, Lawrence, M., Huntington, NY 11743 (US)
(74) Representative: Weiss, Peter, Dr. rer.nat.
(86) International application number: US8904121
(87) International publication number: WO9104310

(56) References cited:
- JP-A-56 159 291
- US-A- 3 514 273
- US-A- 3 640 016
- US-A- 3 837 820
- US-A- 3 876 391
- US-A- 3 902 869
- US-A- 3 948 617
- US-A- 4 002 435
- US-A- 4 046 519
- US-A- 4 158 551
- US-A- 4 162 143
- US-A- 4 224 038
- US-A- 4 226 601
- US-A- 4 230 460
- US-A- 4 270 926
- US-A- 4 445 908
- US-A- 4 456 688
- US-A- 4 477 258
- US-A- 4 616 574
- US-A- 4 801 304

## Description

### CROSS REFERENCE TO RELATED APPLICATIONS

The present application is a continuation-in-part of prior copending applications serial nos. 780,783, and 787,293, which in turn, are a division and a continuation-in-part, respectively, of copending application serial no. 653,808, which, in turn, is a continuation-in-part of application Serial No. 547,892, (which issued as US-A-4,618,348.

### 1. INTRODUCTION

This invention relates to a method according to the first part of claim 1 and in particular for burning high sulfur (S) content combustible compositions, wherein low, environmentally-acceptable, oxidized sulfur compound (SOX) emissions are realized. More particularly, this invention relates to the mixing of high sulfur content compounds with admixtures of soluble and insoluble sulfur sorbents. Use of such admixtures, it has been found, results in a far greater reduction on SOX emissions, than would be expected from the activity of each sorbent used alone, while exhibiting no deleterious effects on the combustion efficiency.

These admixtures can be used to control the SOX emissions from all high S content combustible compositions including hydrocarbon oils and coal/water slurries. Extremely viscous hydrocarbons can be burned as preatomized fuels, i.e., oil-in-water emulsions, the viscosity of which is greatly reduced in comparison with that of the starting hydrocarbon. Thus, a wide array of hydrocarbons previously unsuitable for use due to air pollution constraints can be burned.

### 2. BACKGROUND OF INVENTION

### 2.1. VISCOUS HYDROCARBONS

While large quantities of high-quality, relatively inexpensive, light crude oils presently are recoverable from world-wide geographical locations, ever-increasing consumption of petroleum fuels and other petroleum products and the energy crisis precipitated by such high demands have brought interest to bear on the enormous reserves of low-gravity, viscous hydrocarbons which also exist throughout the world. Viscous hydrocarbons present in natural deposits have been generally classified as viscous crude oils, bitumen or tar and have been variously called heavy crudes, native bitumen, natural bitumen, oil sands, tar sands, bituminous sands or deposits and natural asphalts, all of which materials are chemically gradational and nearly indistinguishable without standardized analyses. [For a discussion of the general characteristics of viscous hydrocarbons and the problem of precisely defining or classifying them, see Meyer, "Introduction" in: The Future of Heavy Crude and Tar Sands, p. 1, Mining Informational Services, McGraw Hill, Inc., New York (1981). See also Section 6.2 infra.]

The geographical distribution of heavy crude reserves is given in Table I [abstracted from Meyer and Dietzman (1981), "World Geography of Heavy Crude Oils," in: The Future of Heavy Crude and Tar Sands, pp. 16-28, Mining Informational Services, McGraw Hill, Inc., New York (1981)]. The total estimated figure for oil in place is 9858 x 10¹¹ ℓ (6200 x 10⁹ barrels). Venezuela heads the list with roughly half of this total, 4770 x 10¹¹ ℓ (3000 x 10⁹ barrels). Canada follows closely with 46905 x 10¹⁰ ℓ (2950 x 10⁹ barrels) (this total includes hydrocarbon in bitumen), while the United States has an estimated 12243 x 10⁹ ℓ (77 x 10⁹ barrels). To put these figures in perspective, the total world reserves of oil lighter than 20°API is estimated to be about 10494 x 10¹⁰ ℓ (660 x 10⁹ barrels). Yet undiscovered reserves are estimated at 1431 x 10¹¹ ℓ (900 x 10⁹ barrels). Thus, heavy crude is more plentiful than conventional oil by about a factor of four.

**TABLE I**

| WORLD HEAVY OIL DEPOSITS (Billions of Liter (Barrels) | | |
|---|---|---|
| Country | Resource | |
| | In-Place | Estimated Recoverable |
| Venezuela | 477000 (3000) | 79500 (500) |
| Canada | 469050 (2950) | 33867 (213) |
| United States | 12243 (77) | 4770 (30) |
| Italy | 1908 (12) | 159 (1) |
| Madagascar | 3975 (25) | 159 (1) |
| Iran | 4611 (29) | 477 (3) |
| Iraq | 1590 (10) | 159 (1) |

It is clear that reserves of conventional light crudes are being depleted much faster than heavy crudes and that development of world reserves of viscous hydrocarbons will eventually become necessary to support world petroleum demands. Significant production of heavy crudes has begun, primarily by steam-assisted enhanced recovery methods. For example, recent estimates place production of heavy crude oil in California at 39.750.000 ℓ (250,000 barrels) per day. Future estimates [Barnea, "The Future of Heavy Crude and Tar Sands," in: The Future of Heavy Crude and Tar Sands, pp. 13-15, Mining Informational Services, McGraw Hill, Inc., New York (1981)] project that by the year 2000, production of heavy oil plus the bitumen from tar sands will increase to one-third of the world's total oil production. Such rapid development of heavy oil resources will extend the petroleum era and should: 1) allow products from heavy crudes to benefit from the existing energy infrastructure; 2) assure fuel supplies to the transportation sector and feed-stock to petrochemical plants; 3) be a stabilizing factor for world petroleum prices, increasing the number of oil producing countries; 4) reduce the strategic and political aspects of oil production; and 5) postpone the need for massive investments in coal conversion and other facilities for synthetic oil production.

### 2.2. COMBUSTION OF OIL-IN-WATER EMULSIONS

The vast majority of combustible emulsions known in the art are water-in-oil emulsions, primarily consisting of relatively small amounts of water (1-10% by volume) in oil to enhance combustion. Some combustible oil-in-water emulsions have been described [see e.g., US-A-3,958,915; 4,273,611 and 4,382,802]. Notably, however, the oil phases used have been light, low viscosity fuels and other low viscosity oils, e.g., kerosene, gasoline, gas oil, fuel oils and other oils which are liquid at room temperature. Combustible thixotropic jet fuels and other safety fuels have been described in US-A-3,352,109; 3,490,237 and 4,084,940. Under resting (stationary) conditions, these oil-in-water emulsions are in the form of gels with apparent rest viscosities of 1000 cps and preferably 50,000-100,000 cps. These thixotropic oil-in-water emulsions exhibit low viscosities under high pumping (high shear) rates.

### 2.3. MICROBIAL SURFACE-ACTIVE COMPOUNDS

Many microbes can utilize hydrocarbon as their sole source of carbon for growth and energy production. The hydrocarbon substrates may be linear, branched, cyclic or aromatic. In order to rapidly assimilate such water-insoluble substrates, the microbes require a large contact area between themselves and the oil. This is achieved by emulsifying the oil in the surrounding aqueous medium. Hydrocarbon degrading microbes frequently synthesize and excrete surface active agents which promote such emulsification.

For example, the growth of Mycobacterium rhodochrous NCIB 9905 on n-decane yields a surface active agent which was reported by R.S. Holdom et al. [J. Appl. Bacteriol. 32, 448 (1969)] to be a nonionic detergent. J. Iguichi et al. [Agric. Biol. Chem., 33, 1657 (1969)] found that Candida petrophilium produced a surface active agent composed of peptides and fatty acid moieties, while T. Suzuki et al. [Agric. Biol. Chem., 33, 1919 (1969)] found trehalose lipid in the oil phase of culture broths of various strains of Arthrobacter, Brevibacterium, Corynebacterium and Nocardia. Wagner has reported the production of trehalose lipids by Nocardia rhodochrous and Mycobacterium phlei and their use in oil recovery [US-A-4,392,892 and 4,286,660].

Torulopsis gropengiesseri was found to produce a sophorose lipid, while rhamnolipids are reported by K. Hisatsuka et al. [Agric. Biol. Chem., 35, 686 (1971)] to have been produced by Pseudomonas aeruginosa strain S7B1 and by S. Itoh et al. [Agric. Biol. Chem., 36, 2233 (1971)] to have been produced by another P. aeruginosa strain, KY4025. The growth of Corynebacterium hydrocarboclastus on kerosene was reported by J.E. Zajic and his associates [Dev. Ind. Microbiol., 12, 87 (1971); Biotechnol. Bioeng., 14, 331 (1972); Chemosphere 1, 51 (1972); Crit. Rev. Microbiol., 5, 39; US-A-3,997,398] to produce an extracellular heteropolysaccharide which, among other properties, emulsified kerosene, Bunker C fuel oil and other fuel oils.

Gutnick et al. discovered that Acinetobacter calcoaceticus ATCC 31012 (previously designated Acinetobacter sp. ATCC 31012 and also called RAG-1) produces interfacially active extracellular protein-associated lipopolysaccharide biopolymers called emulsans. These biopolymers are produced and build up as a capsule or outer layer around the bacterial cell during growth and are eventually released or sloughed off into the medium, from which they can be harvested as extracellular products. Acinetobacter calcoaceticus ATCC 31012 produces α-emulsans when grown on ethanol or fatty acid salts [US-A-4,230,801; 4,234,689 and 4,395,354] and β-emulsans when grown on crude oil or hexadecane [US-A-3,941,692]. The α-emulsans and β-emulsans can be derivatized to an O-deacylated form called psi-emulsans [US-A-4,380,504]. The α-emulsans, β-emulsans and psi-emulsans can be deproteinized to yield apo-α-emulsans, apo-β-emulsans and apo-psi-emulsans, respectively [US-A-4,311,830; 4,311,829 and 4,311,831, respectively].

Cooper and Zajic [Adv. Appl. Microbiol. 26:229-253 (1980)] have reviewed the production of surface active compounds by microorganisms. Some of the surface active agents described are listed in Table II.

**TABLE II**

| MICROBIAL SURFACE ACTIVE COMPOUNDS | |
|---|---|
| STRUCTURAL TYPE | PRODUCING MICROORGANISM(S) |
| Carbohydrates-Lipids | |
| Trehalose-Lipids | Nocardia, Mycobacterium, Corynebacterium, Arthrobacter |
| Rhamnose-Lipids | Pseudomonas aeruginosa |
| Sophorose-Lipids | Torulopsis spp. |
| Polysaccharide-Lipid | Candida tropicalis, Acinetobacter calcoaceticus |

| Amino Acid-Lipids | |
|---|---|
| Lipopeptides | Bacillus, Streptomyces, Corynebacterium, Mycobacterium |
| Ornithine-Lipids | Pseudomonas, Thiobacillus, Agrobacterium, Gluconobacter |
| Phospholipids | Thiobacillus, Corynebacterium, Candida, Micrococcus |
| Fatty Acids/Neutral Lipids | Pseudomonas, Mycococcus, Penicillium, Aspergillus, Acinetobacter, Micrococcus, Candida |

### 2.4. REDUCTION OF SOX IN COMBUSTION GASES

Within the past few years there has been an increasing concern with the immediate and long-term effects of atmospheric pollution produced during the burning of hydrocarbon fuels. During this time, substantial amounts of money and effort have been spent to combat this problem. Additionally, the governmental agencies, on the federal, state, and local levels have issued environmental regulations which severely limit the amount of pollutants which can be released into the atmosphere, consequently forcing users of these fuels to make the choice of burning the more expensive, "clean-burning", fuels or, as the supply of such fuels is shrinking, to seek methods to reduce the emissions released by the combustion of the higher-polluting fuels.

A class of pollutants that has, recently, become a major concern is that of gaseous sulfur compounds such as H₂S, COS, SO₂, SO₃ and the like. When released into the atmosphere, these compounds, it has been postulated, can react with atmospheric moisture and oxygen to form sulfuric acid, which results in "acid rain", severely corrosive precipitation that is detrimental to plant and animal life. For this reason, particularly stringent restrictions have been placed upon the amount of gaseous sulfur compounds, notably the oxidized forms of sulfur produced during sulfur burning, SOX, which can be released into the atmosphere during combustion of fuels. Such restrictions have made it nearly impossible to utilize high sulfur content fuels in standard applications. Since many of the viscous hydrocarbon fuels discussed supra, and much of the world's coal reserves, have high sulfur content, use of a significant portion of the world's petroleum and coal reserves presents difficult environmental and economic problems. As the world's hydrocarbon reserves are shrinking, the use of these other fuels becomes necessary.

For this reason, scientists have attempted to lower the gaseous sulfur emissions of high sulfur content fuels. Three main approaches have been used. In the first, the combustion gases are channelled through an SOX absorbent prior to release into the atmosphere, resulting in reduced SOX levels in the effluent gas. This method, also known as "scrubbing" is the most common method in use today; however, it suffers from the major drawback of requiring significant capital outlay for the design and construction of the system. Nonetheless, this is the principal SOX control method in use today.

An alternative approach involves the removal of the sulfur from the fuel prior to the combustion. This may be accomplished by extracting the sulfur components into solvents having a stronger affinity for the sulfur compounds than the fuel. Such solvents are, however, expensive and often will extract significant amounts of combustible fuel components along with the sulfur. For these reasons, this method has proven to be impractical.

More useful, in the case of petroleum hydrocarbons, is hydrogen addition to convert the sulfur in the sulfur compounds to hydrogen sulfide (H₂S), which can be separated from the petroleum fraction. However, this process also requires significant capital outlay.

In the third approach, the fuel is mixed with sulfur sorbents which act to remove the sulfur and the oxidized sulfur compounds during the combustion process. A particular advantage of this approach is that solid compounds can be utilized as sorbents. Such compounds will remain in the solid phase during combustion, thus facilitating the ultimate collection of the sulfur-sulfur sorbent conjugates. Also, because the reaction occurs in the combustion zone, the temperatures are quite high rendering the sorbent species quite reactive; thus, the kinetics of the absorption are directed in favor of the SOX binding.

A major drawback of this method, however, is the lack of adequate sulfur sorbents, thus making efficient sulfur removal difficult. For example, Cottell (U.S. Patent 3,941,552) found in experiments using coal/water slurries that when lime (CaO) is present in a 50% excess of the stoichiometric requirement (to achieve 100% S removal), a 50% reduction in SOX levels is observed; this increases to 80% when twice the stoichiometric requirement of lime is used. Dooher et al. (Fuel, 59, Dec., 1980, pp. 883-891) conducted burn experiments on water-in-oil emulsions of high sulfur oil utilizing soda ash (Na₂CO₃) as a sorbent and claimed to have found somewhat better results (50% of the stoichiometric requirement of Na₂CO₃ achieved a 45% SO₂ removal). However, in a commercial boiler, the use of high concentrations of sodium salts is undesirable due to the well-known side effect of fouling, which necessitates frequent cleaning of the boiler.

The US-A-4 226 601 relates to a process for preparing a coal or lignite fuel, which contains sulfur, for combustion. A sulfur-containing coal or lignite is reduced in sizes to form a finally devided coal or lignite. The thus pulverized sulfur-containing coal or lignite is then admixed with a finally devided inorganic material. The resulting admixture of coal or lignite and the inorganic material can thereafter be subjected to a combustion process in conventional combustion equipment with reduced emission of sulfur oxide combustion products. The inorganic material that is admixed with a finally devided or pulverized sulfur containing coal or lignite can be at least one material selected from an oxide of sodium, potassium, calcium or barium; a hydroxide of sodium, potassium, calcium or barium; a carbonide of sodium, potassium, calcium or barium; or dolomite. Since large quantities of such inorganic materials will be utilized in the process of this invention, inexpensive sources of such inorganic materials will be very attractive.

There exists, therefore, a real need for efficient and inexpensive sulfur sorbent agents which can effectively limit SOX emmissions, yet which will not exhibit deleterious effects such as fouling.

### 3. Summary of invention:

It is an objective of this invention to provide a method whereby a reduction in the oxidized sulfur (SOX) emissions during the burning of high sulfur content hydrocarbons and coals can be achieved. More particularly, it is an objective of this invention to provide a method whereby sulfur-containing materials, including hydrocarbons, coals, coal/water slurries and hydrocarbon-in-water emulsions, can be burned safely and efficiently, in an environmentally-acceptable manner wherein the SOX emissions are reduced to a value below the permissible local regulatory standard.

It is also an objective of this invention to provide clean burning combustible compositions which, during combustion, will produce lower sulfur emissions than the neat hydrocarbons or coals.

These objects will be solved by the method according to the second part of claim 1.

This invention provides a method for decreasing SOX emissions during combustion of high sulfur content hydrocarbons and coals by adding to such materials an admixture of insoluble and soluble sulfur sorbents prior to the burning. It has been found that, remarkably, this admixture of sulfur sorbents provides a higher degree of SOX emission reduction than would be predicted on the basis of the reduction efficiency of each sorbent individually, i.e., the admixture components exhibit a catalytic effect on the SOX removal efficiency of each other. By use of these sorbents, the SOX emissions during combustion of high sulfur content hydrocarbons (including coals) can be brought within environmentally acceptable levels, making such materials commercially useful.

This invention also provides methods for reducing the SOX emissions during the combustion of viscous, high sulfur content hydrocarbons by forming preatomized fuels (hydrocarbon-in-water emulsions) and adding the insoluble/soluble sorbent admixture to the preatomized fuels. As with the unemulsified fuel compositions described above, the admixture achieves a remarkable reduction in SOX emissions when the preatomized fuel is burned. Similar reductions can be seen using coal/water slurries treated with the sorbents as fuels.

This invention also provides fuel compositions comprised of sulfur-containing combustible compounds, including preatomized fuels and coal slurries, and admixtures of soluble/insoluble sulfur sorbents, which exhibit reduced SOX emissions when burned.

### 4. NOMENCLATURE

The term "hydrocarbosol" is defined as any bioemulsifier-stabilized hydrocarbon-in-water emulsion wherein the individual hydrocarbon droplets are essentially surrounded or covered by water-soluble bioemulsifier molecules predominantly residing at the hydrocarbon/water interface, which bioemulsifier molecules form an effective barrier against droplet coalescence and hence promote the maintenance of discrete hydrocarbon droplets suspended or dispersed in the continuous, low-viscosity aqueous phase.

The term "water-soluble" is defined to include water-dispersible substances.

The term "viscous hydrocarbon" is defined as any naturally occurring crude oil or any residual oil remaining after refining operations which is generally characterized by a viscosity of 10²-10⁶ centipoise or greater and otherwise generally, but not necessarily, characterized by an API gravity of about 20°API or less, high metal content, high sulfur content, high asphaltene content and/or high pour point. The term "viscous hydrocarbon," it is to be understood, also encompasses the following nomenclature: vacuum residuals, vis-breaker residuals, catalytic-cracker residuals, catalytic hydrogenated residuals, coker residuals, ROSE (residual oil supercritical extraction) residuals, tars and cut-back tars, bitumen, pitch and any other terms describing residuals of hydrocarbon processing.

The term "pre-atomized fuel" is defined as any hydrocarbosol and any viscous hydrocarbon-in-water emulsion formed by methods described herein for use as a combustible fuel.

The term "bioemulsifier" is defined as any biologically derived substance which, by virtue of any combination of characteristics including, but not limited to, high molecular weight, polymeric nature, highly specific three-dimensional structure, hydrophobic and hydrophilic moieties and sparing solubility in hydrocarbons, binds tightly to the hydrocarbon/water interface and essentially covers the surface of individual hydrocarbon droplets in hydrocarbon-in-water emulsions, effectively maintaining discrete droplets and preventing coalescence, and thereby imparting substantial stability to hydrocarbon-in-water emulsions. An example of a bioemulsifier is α-emulsan.

The term "biosurfactant" is defined as any biologically derived substance which reduces the interfacial tension between water and a hydrocarbon and, as a result, reduces the energy requirement (mixing energy) for creation of additional interfacial area. An example of a biosurfactant is a glycolipid.

The term "surfactant package" is defined as any composition useful for forming hydrocarbon-in-water emulsions of viscous hydrocarbons generally characterized by a paraffin content of about 50% by weight or less and an aromatic content of about 15% by weight or greater with viscosities of about 100 centipoise or greater at 65,6°C (150°F), which composition may comprise a chemical surfactant or a combination of chemical co-surfactants or a combination of co-surfactant(s) and biosurfactant(s) or a combination of chemical surfactant(s) and bioemulsifier(s) or a combination of chemical surfactant(s), biosurfactant(s) and bioemulsifier(s), and which may also include chemical emulsion stabilizers, and which may be in aqueous form.

The term "emulsans," which reflects the polysaccharide structure of these compounds and the exceptional bioemulsifier activity of these materials, generically identifies those capsular/extracellular microbial protein-associated lipoheteropolysaccharides produced by Acinetobacter calcoaceticus ATCC 31012 and its derivatives or mutants, which may be subdivided into the α-emulsans and the β-emulsans. The name "apoemulsan" generically identifies those deproteinized lipopolysaccharides obtained from the emulsans.

The term "α-emulsans" defines those extracellular microbial protein-associated lipopolysaccharides produced by Acinetobacter calcoaceticus ATCC 31012 and its derivatives or mutants in which the lipopolysaccharide components (i.e., without the associated protein) are completely N-acylated and partially O-acylated heteropolysaccharides made up of major amounts of D-galactosamine and an aminouronic acid, the lipopolysaccharide components containing at least 5 percent by weight of fatty acid esters in which (1) the fatty acids contain from 10 to 18 carbon atoms; and (2) about 50 percent by weight or more of such fatty acids are composed of 2-hydroxydodecanoic acid and 3-hydroxydodecanoic acid. It follows, therefore, that the deproteinized α-emulsan are called "apo-α-emulsans."

The term "β-emulsans" defines those extracellular microbial protein-associated lipopolysaccharides produced by Acinetobacter calcoaceticus ATCC 31012 and its mutants in which the lipopolysaccharide components (i.e., without the associated protein) are completely N-acylated and partially O-acylated heteropolysaccharides made up of major amounts of D-galactosamine and an aminouronic acid, the lipopolysaccharide components containing less than 5 percent by weight of fatty acid esters in which (1) the fatty acids contain from 10 to 18 carbon atoms; and (2) less than 50 percent by weight of such fatty acids are composed of 2-hydroxydodecanoic acid. The deproteinized β-emulsans are called "apo-β-emulsans."

The term "psi-emulsans" defines the O-deacylated extracellular protein-associated microbial polysaccharides obtained from the emulsans, the protein-free components of such psi-emulsans being completely N-acylated heteropolysaccharides made up of major amounts of D-galactosamine and an aminouronic acid and containing from 0 to 1 percent of fatty acid esters in which, when present, the fatty acids contain from 10 to 18 carbon atoms. These protein-free components are called "apo-psi-emulsans," regardless of how they are prepared.

The term "polyanionic heteropolysaccharide biopolymers" defines those biopolymers in which (a) substantially all of the sugar moieties are N-acylated aminosugars, a portion of which is N-acylated-D-galactosamine and another portion of which is N-acylated aminouronic acid, a part of the N-acyl groups of such heteropolysacchardide being N-3-hydroxydodecanoyl groups; and (b) at least 0.2 micromoles per milligram of such heteropolysaccharide consist of fatty acid esters in which (1) the fatty acids contain 10 to 18 carbon atoms and (2) about 50 percent by weight or higher of such fatty acids are composed of 2-hydroxydodecanoic acid and 3-hydroxydodecanoic acid.

The term "SOX" defines all oxidized sulfur compounds produced during sulfur combustion without reference to the degree of oxidation.

The term "hydrocarbon" is defined as any naturally occurring petroleum crude oil, residue, or distillate, including coals.

The term "sulfur containing combustible compound" refers to all combustible compounds which contain measurable quantities of sulfur compounds and which, when burned, produce measurable amounts of SOX.

The term "high sulfur content" includes all compounds which, when burned, have a SOX emission level which exceeds the standard set by the local regulatory authority.

The term "slurry" includes all dispersoids wherein a ground or pulverized solid phase is dispersed in a continuous liquid phase.

### 5. BRIEF DESCRIPTION OF THE FIGURES

FIG. 1 is a graphical representation of the Removal Efficiency as a function of % excess oxygen with the addition of 1% and 2% CaCO₃ as a S sorbent, at 30 and 50% furnace loads.

FIG. 2 is a graphical representation of the Removal Efficiency as a function of the % excess oxygen for three CaCO₃/Na₂CO₃ S sorbent systems at 30 and 50% furnace loads.

FIG. 3 is a graphical representation of the Removal Efficiency as a CaCO₃/10% calcium acetate sorbent system at a 30 and 50% furnace load.

### 6. DETAILED DESCRIPTION OF THE INVENTION

### 6.1. SURFACTANT PACKAGES

The surfactant packages suitable for forming preatomized fuels can be formulated with a wide variety of chemical and microbial surface active agents and are preferably formulated with water-soluble surface active agents to provide for the formation of oil-in-water, as opposed to water-in-oil, emulsions. The surfactant packages can be formulated with numerous chemical surfactants, used alone or in conjunction with chemical co-surfactants of the same type (e.g., a combination of water-soluble nonionic surfactants) or of different types (e.g., a combination of water-soluble nonionic, anionic, cationic and/or amphoteric surfactants), and can be further formulated in combination with (a) a water-soluble biosurfactant or combination of biosurfactants as co-surfactant(s) and/or (b) a water-soluble bioemulsifier or combination of bioemulsifiers as emulsion stabilizer(s). In certain instances, chemical emulsion stabilizers may also be used in place of bioemulsifiers. It is also possible to formulate surfactant packages comprising only microbial surface active agents, i.e., combinations of biosurfactants and bioemulsifiers. The surfactant packages vary with the type of viscous oil to be emulsified. The following general compositions are offered by way of illustration. For viscous crudes, surfactant packages can be formulated to comprise at least one chemical surfactant and at least one bioemulsifier. They can also be formulated to comprise at least one water-soluble nonionic surfactant, at least one water-soluble anionic surfactant, and at least one bioemulsifier. For viscous crudes or viscous residuals, surfactant packages can be formulated to comprise at least one water-soluble non-ionic surfactant or at least one anionic surfactant or combinations of non-ionic surfactants and anionic surfactants and which can further comprise biosurfactants and/or bioemulsifiers.

The types of water-soluble nonionic chemical surfactants suitable for use in the surfactant packages are listed in Table III.

In surfactant packages for viscous crudes, the preferred water-soluble nonionic chemical surfactants are ethoxylated alkyl phenols and ethoxylated alcohols. In surfactant packages for viscous residuals, the preferred water-soluble nonionic surfactants are, again, ethoxylated alkyl phenols and also polyoxyalkylated amines. The ethoxylated alkyl phenols are of the general formula:

RₓC₆H₄(OC₂H₄)ₙOH

wherein R represents an alkyl group containing from 8 to 12 carbon atoms (i.e., about C₈ to about C₁₂), x represents the number of alkyl groups and is either 1 or 2, and wherein n represents the number of ethoxy groups (moles ethylene oxide) which can range from 1 to 100. [For a list of commercially available ethoxylated alkylphenols, see "Surfactants and Detersive Systems" in: Encyclopedia of Chemical Technology, Kirk-Othmer (Third Edition), Volume 22, pp. 366-367, John Wiley & Sons, New York (1983).] In surfactant packages for viscous crudes, preferred ethoxylated alkyl phenols are those having R groups of 8 or 9 carbon atoms and having from about 7 to about 100 ethoxy groups. An example of a particularly preferred ethoxylated alkyl phenol is monononylphenol with about 40 ethoxy groups.

The ethoxylated alcohols are of the general formula:

R(OC₂H₄)ₙOH

wherein R represents an aliphatic group (linear or branched) containing from 6 to 18 carbon atoms and wherein n represents the number of ethoxy groups which can range from 2 to 100. [For a list of commercially available ethoxylated alcohols, see "Surfactants and Detersive Systems" in: Encyclopedia of Chemical Technology, supra, pp. 364-365.] Examples of ethoxylated alcohols include ethoxylated trimethylnonanols with 3 to 9 ethoxy groups and ethoxylated secondary alcohols having R groups of 11 to 15 carbon atoms with 3 to 30 ethoxy groups, but preferably greater than about 7 ethoxy groups.

The polyoxyalkylated amines are of the general formula:

RₓN_{y}(CH₂)₂

wherein R represents an oxyalkyl group containing either 2 or 3 carbon atoms. These R groups can range in number from 4 to 500, and that number is represented by x. The number of amine groups is represented by y and the alkyl group is preferably ethyl (C₂H₄). Preferred polyoxyalkylated amines are those having R groups of 2 or 3 carbon atoms and having from 50 to 450 oxyalkyl groups. An example of a particularly preferred polyoxyalkylated amine is a polyoxyalkylated diamine with about 50 ethoxy groups and about 60 propoxy groups.

The types of water-soluble anionic chemical surfactants suitable for use in the surfactant packages are listed in Table IV.

In surfactant packages for both viscous crudes and viscous residuals, the preferred water-soluble anionic chemical surfactants are sulfonated or sulfated forms of nonionic surfactants. In surfactant packages for viscous crudes, ethoxylated alcohol sulfates are preferred. In surfactant packages for viscous residuals, sulfonated or sulfated ethoxylated alkylphenols and ethoxylated alcohol sulfates are preferred. In surfactant packages for both viscous crudes and viscous residuals, alkylaryl sulfonates are also preferred anionic chemical surfactants. The ethoxylated and sulfated alcohols are of the general formula:

R(OC₂H₄)ₙOSO₃M

wherein R represents an aliphatic group containing from 6 to 16 carbon atoms, preferably from 12 to 14, n represents the number of ethoxy groups which can range from 1 to 4, preferably from 2 to 3, and M includes, but is not limited to, ammonium (NH4), sodium (Na), potassium (K), calcium (Ca) or triethanolamine, preferably ammonium. [For a list of commercially available ethoxylated alcohol sulfates, see "Surfactants and Detersive Systems" in: Encyclopedia of Chemical Technology, supra, p. 357.] The alcohol moiety of the ethoxylated alcohol sulfate can be an even or odd number or mixture thereof. In surfactant packages for viscous crudes, an example of a particularly preferred ethoxylated alcohol sulfate is poly(3)ethoxy C₁₂-C₁₄ linear primary alcohol sulfate, ammonium salt. It is also possible to use nonethoxylated alcohol sulfates, i.e., alcohol sulfates of the formula R(OC₂H₄)ₙOSO₃M as described supra but wherein n = 0. In surfactant packages for viscous residuals, an example of a particularly preferred nonethoxylated alcohol sulfate is the sodium salt of a sulfated lauryl alcohol.

The sulfated ethoxylated alkylphenols are of the general formula:

RC₆H₄(OC₂H₄)ₙOSO₃M

wherein R represents an aliphatic group containing at least 8 or 9 carbon atoms, n represents the number of ethoxy groups which can range from 1 to 100, preferably from about 4 to about 9 and M includes, but is not limited to, ammonium (NH⁺₄), sodium (Na⁺), potassium (K⁺) and calcium (Ca⁺⁺) or triethanoloamine (TEA), preferably ammonium.

An example of a particularly preferred sulfated ethoxylated alkylphenol is the ammonium salt of a sulfated nonylphenol ethoxylate containing, but not limited to, about 4 ethoxy groups.

The alkylaryl sulfonates are of the general formula:

RₙArₘ(SO₃)ₓM

wherein Ar is an aromatic group which is benzyl, naphthyl, phenyl, tolyl, xylyl or ethylphenyl, R is a linear or branched chain alkyl group containing from 2 to 16 carbon atoms, n is 1 or 2, m is 1 or greater, x is at least about 1, and M includes, but is not limited to, ammonium, sodium, potassium, calcium or triethanolamine. [For a list of commercially available alkylaryl sulfonates, see "Surfactants and Detersive Systems" in: Encyclopedia of Chemical Technology, supra, p. 358.] An example of an alkylaryl sulfonate is a modified amine dodecylbenzene sulfonate. In surfactant packages for viscous residuals, an example of a particularly preferred alkylaryl sulfonate is the sodium salt of polymerized alkylnaphthalene sulfonate.

The preferred water-soluble microbial surface active agents for use in the surfactant packages are any microbial or other biologically-derived substances which function as bioemulsifiers, i.e., substances which, by virtue of such characteristics as large molecular weight, polymeric nature, highly specific three-dimensional structure, hydrophobic and hydrophilic nature, and sparing solubility in oil, effectively cover the oil/water interface maintaining discrete, individual oil droplets in oil-in-water emulsions thereby substantially stabilizing emulsions from coalescence. Among the preferred bioemulsifiers are heteropolysaccharide biopolymers produced by bacteria of the genus Acinetobacter and the genus Arthrobacter, and in particular, those produced by strains of Acinetobacter calcoaceticus. Such Acinetobacter heteropolysaccharide biopolymers include, but are not limited to, polyanionic heteropolysaccharide biopolymers, α-emulsans, β-emulsans, psi-emulsans, apo-α-emulsans, apo-β-emulsans and apo-psi-emulsans produced by Acinetobacter calcoaceticus ATCC 31012 (deposited at the American Type Culture Collection in Rockville, MD) defined in Section 4 and described in US-A 4,395,353; 4,395,354; 3,941,692; 4,380,504; 4,311,830; 4,311,829; and 4,311,831, respectively. Other Acinetobacter calcoaceticus materials that can be used are the products of strains NS-1 (NRRL B-15847), NS-4 (NRRL B-15848), NS-5 (NRRL B-15849), NS-6 (NRRL B-15860) and NS-7 (NRRL B-15850). The foregoing "NS" strains have been deposited at the Northern Regional Research Center in Peoria, IL and have been assigned the foregoing NRRL accession numbers. The "NS" strains of Acinetobacter calcoaceticus are described by Sar and Rosenberg, Current Microbiol. 9(6):309-314 (1983). Other Acinetobacter heteropolysaccharide biopolymers are those produced by Acinetobacter calcoaceticus BD4 [Taylor and Juni, J. Bacteriol. 81: 688-693 (1961)]. Particularly preferred Acinetobacter heteropolysaccharide biopolymers are the α-emulsans, the production of which is further described in US-A-4,230,801 and 4,234,689. The α-emulsans are characterized by a Specific Emulsification Activity of about 200 units per milligram or higher, where one unit per milligram of Specific Emulsification Activity is defined as that amount of emulsifying activity per milligram of bioemulsifier which yields 100 Klett absorption units using a standard hydrocarbon mixture consisting of 0.1 ml of 1:1 (v/v) hexadecane/2-methylnaphthalene and 7.5 ml of Tris-Magnesium buffer.

The foregoing Acinetobacter bioemulsifiers can be used in the surfactant packages in a variety of forms including, but not limited to, post-fermentation whole broth; cell-free (Millipore-filtered, e.g.) or partially cell-free supernatants of post-fermentation culture broth; the cells themselves; protease-treated, liquid or dried materials; and protease-treated, ultrafiltered, liquid or dried materials.

Numerous other microbial organisms may possibly serve as a source of biological surface active agents, including biosurfactants and bioemulsifiers, for use in the surfactant packages. Some of these microorganisms and the types of compounds they produce are listed in Table V, though the list is not exhaustive. The surfactant packages may also be formulated with water-soluble cationic chemical surfactants, including, but not limited to, oxygen-free amines, oxygen-containing amines, amide-linked amines and quaternary ammonium salts. Use of cationic chemical surfactants in conjunction with microbial surface active agents would require that the charge characteristic of the biological compounds be considered. For example, cationic chemical surfactants would probably best be used in conjunction with neutral microbial surface active agents and would probably best not be used in conjunction with the preferred polyanionic heteropolysaccharide bioemulsifiers.

Surfactant packages can be formulated from nonionic chemical surfactants or combinations of nonionic and anionic chemical surfactants without bioemulsifiers but preferably, for emulsion stabilization, with bioemulsifiers in the range of 1% to 50% by weight. Surfactant packages comprising bioemulsifiers in the range of 10% to 20% by weight and particularly around 15% by weight are preferred.

### 6.2. VISCOUS CRUDE OILS AND RESIDUAL OILS

Surfactant package compositions can be used to emulsify or emulsify and substantially stabilize numerous viscous hydrocarbons in oil-in-water emulsions which may be directly burned. Viscous hydrocarbons encompass naturally-occuring viscous crude oils (also called heavy crude oils) as well as residual bottom-of-the-barrel products from refineries, such as vacuum resid, other residual fuel oils and asphalt. [See Section 4, Nomenclature, supra.] While low gravity does not necessarily coincide with high density, these characteristics are generally correlated in viscous hydrocarbons.

Generally, the following characteristics are considered typical of the types of crude oils and residual oils:
1. Low API gravity, generally at or below about 20°API. This is the most frequently used criterion, both because it is easily measured and because 20°API crude roughly corresponds to the lower limit recoverable with conventional production techniques.
2. Viscosities in the range of 10² to 10⁶ centipoise (cp) or even higher in some cases.
3. High metal contents. For example, heavy crudes often have nickel and vanadium contents as high as 500 ppm.
4. High sulfur content.
5. High asphaltene content.
6. High pour point.
It is to be noted, of course, that lighter crudes may also be emulsified and/or stabilized with surfactant packages, and such emulsion formation, to yield preatomized fuels, often aids in the handling and combustion of these materials. Since lighter crudes can also contain measurable quantities of sulfur, the use of formation of preatomized fuels from these lighter oils may be useful for the purposes of this invention.

These viscous hydrocarbons which can be emulsified with the surfactant packages and which are most useful to emulsify for transportation and/or burning purposes can be generally defined as having a paraffin content of about 50% by weight or less and an aromatic content of about 15% by weight or greater with viscosities of about 100 centipoise or greater at 65,6°C (150°F). The viscous residuals generally are characterized by a paraffin content in the range from 4% to 40% by weight, an aromatic content in the range from 15% to 70% by weight and an asphaltene content from 5% to 80% by weight.

More specifically, the types of crude oils that can be successfully emulsified and stabilized with surfactant packages include Boscan (Venezuela) crude, an east Texas crude, Jibaro and Bartra (Peru) crudes, El Jobo (Venezuela) crude, and a Kansas crude. The specific viscous residuals that can be successfully emulsified and stabilized with surfactant packages include California vacuum resid, Oklahoma vacuum resid, German visbreaker resid, Texas visbreaker resid, catalytic hydrogenated resid, ROSE bottoms, cutback tar, pyrolysis pitch, and propane deasphalted tar.

Furthermore, residual fuel oils such as those classified as ASTM Grade Number 6 Oils can also be emulsified. Number 6 oils, sometimes referred to as "Bunker C" oils, are high-viscosity oils used mostly in commercial and industrial heating. Their utilization normally requires preheating in the storage tank to permit pumping, and additional preheating at the burner to permit atomizing. The extra equipment and maintenance required to handle Number 6 fuels in nonemulsified form usually precludes its use in small installations. The ASTM standard specifications for Number 6 fuel oils are summarized in Table VI ["Standard Specification for Fuel Oils," ASTM Designation D396-80, in: 1981 Book of ASTM standards, Part 23].

**TABLE VI**

| DETAILED REQUIREMENTS FOR NUMBER 6 FUEL OILS | | |
|---|---|---|
| | Grade of Fuel Oil (No.6, Preheating Required for Burning and Handling) | |
| | Minimum | Maximum |
| Flash Point, °C (°F) | 60 (140) | |
| Water and Sediment, Vol % | | 2.00² |

| Saybolt Viscosity, s¹ | | |
|---|---|---|
| Universal at 38°C (100°F) | ( 900) | (9000) |
| Furol at 50°C (122°F) | ( 45) | (300) |
| Kinematic Viscosity, cSt¹ At 50°C (122°F) | 92 | 638 |

| | | |
|---|---|---|
| ¹ Viscosity values in parentheses are for information only and not necessarily limiting. | | |
| ² The amount of water by distillation plus the sediment by extraction shall not exceed 2.00%. The amount of sediment by extraction shall not exceed 0.50%. A deduction in quantity shall be made for all water and sediment in excess of 1.0%. | | |

### 6.3. EMULSION FORMATION

The surfactant packages of Section 6.1 can be used to form oil-in-water emulsions containing as much as about 90% by volume of the hydrocarbons described in Section 6.2. The aqueous phase into which the hydrocarbon is emulsified can be deionized water, water from a municipal source, or any water, even water with relatively large amounts of dissolved solids such as connate waters or brines, normally located in proximity to oil production, transportation or utilization sites. The aqueous phase can also be an alcohol/water mixture such as methanol/water, ethanol/water or other lower alkanol/water mixtures, and may further contain additives such as anti-corrosion agents, anti-pollution agents or combustion improvers. Oil-in-water emulsions preferably contain oil/water ratios of 50/50 to 80/20, and more preferably from 60/40 to 75/25.

In forming oil-in-water emulsions, it is economically desirable to use as little of the surfactant package as possible while maintaining acceptable emulsion characteristics to suit the particular transportation or utilization requirements. The surfactant packages of Section 6.1 can be used in proportions of surfactant package:hydrocarbon from 1:100 to 1:2,000 by weight. The proportion used can depend on the type of hydrocarbon to be emulsified and/or the purpose for emulsifying it.

Oil-in-water emulsion formation can be brought about by any number of suitable procedures. For example, the aqueous phase containing an effective amount of surfactant package can be contacted with the hydrocarbon phase by metered injection just prior to a suitable mixing device. Metering is preferably maintained such that the desired hydrocarbon/water ratio remains relatively constant. Mixing devices such as pump assemblies or in-line static mixers can be used to provide sufficient agitation to cause emulsification. As a more specific example, for the transportation or utilization of residual oils, it may be possible to emulsify the hot residual oil in about 30% aqueous phase (v/v) with one of the surfactant packages of Section 6.1 as it exits the vacuum still of a refinery.

### 6.3.1. FORMATION OF PRE-ATOMIZED FUELS AT HIGH TEMPERATURES

Some low gravity residual hydrocarbons are extremely viscous and require very high temperatures to make them fluid enough to handle. Such hydrocarbons can be characterized by a viscosity greater than about 1000 cp at 212°F. Maintaining such high temperatures is not economically feasible for the long term storage and transportation of these hydrocarbons. Also, it is not economically feasible to blend these viscous hydrocarbons with much lighter oils (cutter stock) due to either the quantity of lighter oil required to achieve a viscosity which can be handled or the unfavorable characteristics of the viscous hydrocarbon which do not allow for homogeneous blending of lighter oils.

A novel approach to handling extremely viscous hydrocarbons is the stable dispersion of such viscous hydrocarbons into water to form pre-atomized fuels. Pre-atomized fuel formation is achieved by heating the viscous hydrocarbon to a high temperature in order to make it fluid. The hot hydrocarbon phase is brought in contact with the aqueous phase containing appropriate surfactants and/or stabilizers as described in Section 6.1. A key to achieving successful pre-atomized fuel formation is the maintenance of pressure throughout the entire process such that the aqueous phase is not allowed to vaporize. By maintaining the appropriate pressure, i.e., the pressure required to prevent the water in the aqueous phase from boiling, the aqueous phase remains in a liquid state, thus allowing the stable dispersion of the hydrocarbon phase into a continuous water phase. The resulting hot pre-atomized fuel may be rapidly cooled using an appropriate heat exchange device so that the outlet temperature of the pre-atomized fuel is below the vaporization temperature of the aqueous phase at ambient pressure. Alternatively, the pressure may be reduced and the mixture cooled by flashing a portion of the water contained in the pre-atomized fuel.

### 6.3.2. FORMATION OF PRE-ATOMIZED FUELS USING A THERMALLY CRACKED HYDROCARBON DISCHARGE

As is generally known in the refining industry, residual hydrocarbons obtained from the discharge of thermal cracking units have presented unusual problems. The extreme conditions required in processing to obtain greater quantities of high gravity hydrocarbons have resulted in resids which are very susceptible to separation into distinct, non-mixable fractions. The reasons for the occurrence of this phenomenon are not fully known; however, it is believed that the destabilization of high molecular weight components such as asphaltenes is a contributing factor. When such hydrocarbons are used to form pre-atomized fuels as described in Section 6.3., the resulting oil-in-water emulsion may separate into three phases after a short period of static storage. These phases consist of a low API gravity hydrocarbon bottom phase, a water/surfactant middle phase, and a high API gravity hydrocarbon upper phase. Without wishing to be bound or restricted by any particular theory, applicants theorize that the separation may be due to the slow cooling of the pre-atomized fuel which allows sufficient time for the occurrence of complex interactions that may be attributed to both "sticky state" and Ostwald ripening phenomena. The tendency toward separation can be decreased by the use of an appropriate heat exchange device or method to rapidly quench the freshly formed pre-atomized fuel to a temperature at least about 38°C (100°F) below the softening point of the hydrocarbon. By rapidly quenching the oil-in-water emulsion as it exits the mixing unit, a stable pre-atomized fuel is achieved that does not separate with time. It is further theorized that the rapid cooling of the hot pre-atomized fuel does not allow sufficient time for the complex interactions stated above to occur.

### 6.3.3. MIXING OF A SLURRY WITH A PRE-ATOMIZED FUEL

An economical way to increase the btu content of a liquid fuel is achieved by incorporating a high softening point hydrocarbonaceous material (such as coal, coke, ROSE residual, etc.) into a lower softening point fuel. This is usually accomplished by grinding a high softening point hydrocarbon to form very small particles (usually approximately 100 »m in size) and then, dispersing the solid particles in the liquid fuel. The dispersion of a solid in a liquid, however, usually results in the production of a fuel with unfavorable characteristics such as increased viscosity.

A novel method of economically utilizing a high softening point hydrocarbonaceous material (such as coal, coke, ROSE residual, etc.) is achieved by incorporating it into a pre-atomized fuel. This is accomplished by first grinding a material of high softening Point to form very small particles (generally less than about 30 »m) and then forming a slurry by dispersing the particles in a continuous aqueous phase containing a pre-atomized fuel-compatible surfactant package.

The slurry of dispersed particles is mixed at an appropriate ratio with a pre-atomized fuel formulated from a hydrocarbon other than that used to form the slurry. The mixing of a slurry with a pre-atomized fuel results in a liquid fuel which has a viscosity lower than either the slurry or the pre-atomized fuel prior to mixing. The reasons for the reduced viscosity observed in a slurry/pre-atomized fuel mixture are not fully known; however, without wishing to be bound or restricted by any particular theory, applicants believe that the reduction of particle-to-particle interaction is a contributing factor.

### 6.4. PROPERTIES OF EMULSAN-STABILIZED HYDROCARBOSOLS

The hydrocarbon droplets of hydrocarbon-in-water emulsions generally rise to the surface and "float" on the aqueous phase in a process known as creaming, provided the density of the hydrocarbon phase is less than that of the aqueous phase and the droplets in the dispersed phase are too big to be stabilized by Brownian motion. If the "cream" remains undisturbed for a given period of time, the droplets coalesce, giving rise to two separate phases. The emulsans, particularly α-emulsan, are extremely effective in retarding coalescence and the emulsan-stabilized droplets in the "cream" are easily redispersible in the aqueous phase.

The principal factors controlling emulsion stability are electrostatic (charge) effects and steric effects. The properties of emulsans lend themselves to optimal exploitation of these mechanisms. Their large molecular weight and highly specific three-dimensional structure result in an efficient coverage of the hydrocarbon/water interface. This effectively prevents oil-to-oil contact when collisions occur between adjacent droplets. Simultaneously, the polyanionic nature of emulsans causes the surfaces of emulsion droplets to be negatively charged which creates repulsive forces and significantly decreases the collision frequency between hydrocarbon droplets. In addition, the absence of multimolecular emulsan micelles in the water phase and the lack of emulsan solubility in the hydrocarbon phase provides an efficient migration and attachment of the emulsan molecules to the oil/water interface. The overall chemical requirements for emulsion stabilization thus become very small and directly related to the oil droplet size, i.e., interfacial area desired.

### 6.5. BLENDING OF HYDROCARBONS

In some cases hydrocarbons may be too viscous for conventional processing or have characteristics (i.e., low gravity; excessive paraffinic, aromatic, and/or asphaltic contents; etc.) which make them unfavorable to incorporate into stable pre-atomized fuels. One method to reduce viscosity for processing or alleviate unfavorable characteristics is blending the unfavorable hydrocarbon with one which is favorable resulting in a hydrocarbon having characteristics suitable for pre-atomized fuel formation. In this way an otherwise unusable hydrocarbon can be "adjusted" to a usable form.

### 6.6. REDUCTION OF OXIDIZED SULFUR COMPOUND (SOX) LEVELS IN COMBUSTION GASES

### 6.6.1. HIGH SULFUR CONTENT COMBUSTIBLE COMPOUNDS

A large array of naturally occuring hydrocarbon and coal compositions contain appreciable quantities of sulfur (S) as contaminants. When, upon combustion, such fuels produce levels of oxidized sulfur compounds (SOX) in excess of the locally acceptable standard, such fuels are called "high sulfur content" fuels. These fuels cannot be burned in an environmentally acceptable manner without taking steps to reduce these SOX levels.

Combustible compounds which have high S content include, but are not limited to, coals, especially the softer or bituminous coals, and the heavier petroleum fractions such as heavy crude oils, asphalts, resids, bottoms, and tars (see sec. 6.2 supra.). Such compounds cannot be commercially used as fuels without reducing the SOX emissions. As the supply of the "clean burning" or low S fuels is diminished, it is anticipated that these high S fuels will become increasingly important as energy sources.

### 6.6.2. SOLID SULFUR SORBENTS

A wide array of inorganic and organic salts can be used as sulfur sorbents which result in SOX reduction in combustion gases (often, the SOX can be reduced to acceptable levels as defined by local regulatory standards thereby making the fuels "clean burning"). Such compounds react with the oxidized sulfur at some time during the combustion process to form the corresponding sulfates and sulfites. A particular advantage of reacting during the combustion process is that, at the high temperatures realized within and in the vicinity of flame, the sorbents become highly reactive species and the kinetics of the reaction strongly favor the binding of the SOX.

A major factor in determining the sorbent efficiency is the actual physical particle size, as only exposed surfaces will be reactive. As the particle size decreases, the surface area per unit mass of sorbent increases, causing the efficiency to increase. It is, therefore, desirable to achieve as small a particle size as practical.

Sorbents can be conveniently divided into two classes based on their water solubility: soluble sulfur sorbents and insoluble sulfur sorbents. The insoluble sulfur sorbents are generally the less expensive of the two, but their efficiency is usually not as great.

This low efficiency is due primarily to the fact that the particle size of the insoluble sorbents is determined by physical processes such as grinding. Thus, a practical limit exists for the minimum particle size and the efficiency is, therefore, also limited. The insoluble sorbents are generally found in abundance naturally and include the alkaline earth metal carbonates such as calcium carbonate (CaCO₃, limestone) and magnesium carbonate (MgCO₃). Minerals containing high quantities of these compounds such as dolomite (a mixture of CaCO₃ and MgCO₃) are also useful as sorbents. A primary criterion for the selection of an insoluble sorbent is that it be relatively inexpensive, since its efficiency will be low.

The soluble sorbents, on the other hand, are generally more expensive. Included in this category are calcium, sodium, and magnesium salts of formate, acetate, propionate and higher organic radicals. Another soluble sorbent, sodium carbonate (soda ash, Na₂CO₃) is much less expensive than any of the organic salts, but this compound suffers from the drawback of causing boiler fouling, greatly limiting its utility in commercial applications.

The soluble sorbents are generally much more efficient in reducing SOX emissions than the insoluble sorbents, particularly in fuels where water forms a significant component of the mixture, such as in coal/water slurries or preatomized fuels (where water is the continuous phase). In these compounds, it has been postulated that the dissolution of the soluble salts greatly reduces the effective particle size of the sorbent, which increases the efficiency. Since the particle size is not dependent on physical processes, the effective particle size can be much lower and the efficiency much higher than achievable with insoluble sorbents. The high cost of soluble sorbents, however, is a major drawback to their use.

### 6.6.3. MIXED SOLUBLE/INSOLUBLE SORBENT PACKAGES

Admixtures of soluble and insoluble sorbents can be utilized to achieve highly efficient SOX reduction during combustion of high sulfur content fuels including preatomized fuels and coal/water slurries. These admixtures, it has been discovered, exhibit a remarkable reduction in SOX levels; in fact, the SOX reduction efficiency of the admixture exceeds the combined efficiency of each component separately. Apparently each component exerts a catalytic effect on the SOX absorbing ability of the other.

While not wishing to be bound by theory, applicants postulate that this effect arises from interactions between the soluble and insoluble absorbents both prior to and during the combustion which renders the insoluble species more reactive, enhancing the overall efficiency of the admixture. In this way, the benefit of the high efficiency of the soluble sorbents can be combined with the low cost of insoluble sorbents, making a efficient and cost-effective SOX reduction system.

In the admixtures themselves, the quantity of soluble sorbents required to achieve this effect is quite small, depending on the particular sorbents used. Generally, a concentration of soluble sorbent ranging from 0.5-20% (by weight) and, preferably, from 1-10% in the admixture will produce a reduction in SOX levels sufficient to meet the local environmental standards. Since the admixture greatly increases the SOX reduction efficiency as compared with either sorbent alone, the concentration of the admixture in the fuel can also be kept low, generally 0.5-25% (by weight). Thus, the amount of sorbent admixture used is quite low for the SOX reduction observed.

In one embodiment, an admixture of 90% CaCO₃ and 10% CaAc (calcium acetate) was found to exhibit a removal efficiency (a measurement of the theoretical SOX reducing capacity to the actual SOX reduction observed) of 31-44% for a sulfur-containing resid. Even when this amount is corrected for the presence of CaAc by assuming the CaAc reacted with sulfur with 100% efficiency, (a very conservative estimate since, alone, it exhibits a removal efficiency of 50%), the removal efficiency is still 26-40%, as compared with 9-19% observed with an equivalent amount of calcium carbonate as the only sorbent and making the comparison under similar operating conditions. Thus, the SOX reducing capacity is greatly enhanced by forming the admixture.

In another embodiment, the sorbent admixture can be added to coal, either in a water slurry or solid form, resulting in reduced SOX emissions. Since, as stated supra, large amount of coal reserves have high sulfur content, the invention permits the coal to be burned in an-environmentally acceptable manner.

Additionally, the use of these solid sorbent admixtures confers the benefit of permitting easy collection and removal of the bound sulfate and sulfite, since they are in the solid phase. In fact, when calcium sorbents are used, the result is CaSO₄ (gypsum) which is industrially useful. Thus, the potential for adverse environmental effects (due to waste disposal) is further reduced.

### 7. EXAMPLES

### 7.1. PREPARATION OF BIOEMULSIFIERS

### 7.1.1. PREPARATION OF TECHNICAL GRADE α-EMULSAN

The α-emulsans produced by Acinetobacter calcoaceticus ATCC 31012 during fermentation on ethanol are known bioemulsifiers as described in US-A-4,395,354. The α-emulsans used in the experiments described infra were technical grade materials (unless otherwise indicated) which were prepared in either of two ways. Both methods of preparation involved enzyme treatment and drying but differed in the order in which these steps were performed. By one method, centrifuged (approximately 90% cell-free) fermentation broth containing α-emulsans resulting from a fermentation of Acinetobacter calcoaceticus ATCC 31012 in ethanol medium was drum-dried and the resulting material was treated in the following manner prior to use. A 10% by weight suspension of the material, so-called technical grade α-emulsan, was prepared in deionized water and heated to 50°-60°C while continuously stirring. The pH of the suspension was adjusted to pH 8.5 by adding 50% by weight sodium hydroxide (diluted, if necessary). Protease enzyme (NOVO Industries, 1.5M Alcalase) was added at a level of 1 part protease:500 parts solid α-emulsan. The mixture was allowed to remain at 50°-60°C while being stirred for about three hours. Reactions were run to completion as judged by the absence of visible precipitable emulsan following centrifugation of the reaction mixture. After completion of the enzyme treatment, the reaction mixtures were raised to approximately 70°C to denature the protease and stop its activity. The solutions were cooled to room temperature and Cosan PMA-30 (Cosan Corporation), a preservative, was added at a level of 1 part Cosan:500 parts α-emulsan solution.

By another method, enzyme treatment of the α-emulsan was performed prior to drum drying according to the folowing protocol. Fermentation broth containing α-emulsan resulting from a fermentation of Acinetobacter calcoaceticus ATCC 31012 in ethanol medium was centrifuged to remove approximately 90% of the bacterial cells. To the centrifuged broth, protease enzyme (as previously described) was added in a ratio of 1 gram protease:500 units per milligram of Specific Emulsification Activity (where one unit per milligram of Specific Emulsification Activity is defined as that amount of emulsifying activity per milligram of bioemulsifier which yields 100 Klett absorption units using a standard hydrocarbon mixture consisting of 0.1 ml of 1:1 (v/v) hexadecane/2-methylnaphthalene and 7.5 ml of Tris-Magnesium buffer). The protease reaction was run to completion as described supra. The protease-treated centrifuged broth was then evaporated to a 10% (w/v) slurry of α-emulsan. The slurry was sprayed dried and the resulting material is also referred to as technical grade α-emulsan.

### 7.1.2. ADDITIONAL PREPARATIONS OF ACINETOBACTER CALCOACETICUS BIOEMULSIFIERS

Fermentations of Acinetobacter calcoaceticus ATCC 31012 were run on ethanol as described in US-A-4,395,354. The following fractions of the resulting broth were used to formulate surfactant packages: whole broth, supernatants, cells, enzyme-treated whole broth, enzyme-treated supernatants, enzyme-treated cells (where the enzyme treatment was as described for the second method in Section 7.1.1. supra), homogenized cells, boiled cells, and so-called "Millipore emulsan." Millipore emulsan is prepared by Millipore filtering whole broth to remove cells, followed by enzyme treatment (described supra) and ultrafiltration. The foregoing preparations were used in liquid or wet form. The Millipore emulsan samples can be further dialyzed against ammonium bicarbonate and freeze-dried prior to use in surfactant packages.

Whole broth and enzyme-treated whole broth from fermentations of Acinetobacter calcoaceticus ATCC 31012 on soap stock (run under conditions similar to those described in US-A-4,230,801), were also used.

Acinetobacter calcoaceticus NS-1 (NRRL B-15847) was grown in a fermentor on ethanol medium under conditions similar to those described in US-A-No. 4,395,354. Both whole broth and enzyme-treated whole broth were used to formulate surfactant packages.

Acinetobacter calcoaceticus strains NS-4 (NRRL B-15848), NS-5 (NRRL B-15849), NS-6 (NRRL B-15860) and NS-7 (NRRL B-15850) were grown for 3 days in shake flask cultures in 2% ethanol medium as described US-A-4,395,354. Enzyme-treated whole broth samples were prepared from the NS-4, NS-5 and NS-7 cultures. Enzyme-treated supernatant samples were prepared from NS-4, NS-5, NS-6 and NS-7 cultures. These preparations were also used to formulate surfactant packages.

### 7.2. HYDROCARBON CHARACTERISTICS

### 7.2.1. BOSCAN CRUDE OIL

Boscan crude oil is a heavy crude produced from the oilfields of western Venezuela. The characteristics of the crude, its specific gravity, API gravity (°API), paraffin content (% by weight), aromatic content (% by weight), asphaltene content (% by weight) and viscosity (in centipoise) versus temperature (degrees Celsius (Fahrenheit) profile, were determined experimentally and are summarized in Table VII. The paraffin, aromatic, sulfur and asphaltene content were determined by the methods described in Section 7.2.3.

**TABLE VII**

| BOSCAN CRUDE OIL CHARACTERISTICS | |
|---|---|
| Specific Gravity | = 0.983 |
| API Gravity (calculated) | = 12.5°API |
| Paraffin content | = 18.0% (w/w) |
| Aromatic content | = 60.0% (w/w) |
| Asphaltene content | = 22.0% (w/w) |
| Sulfur content | = 5.8% (w/w) |

| Viscosity (cp) | Temperature °C (°F) |
|---|---|
| 4,500 | 60 (140) |
| 24,000 | 38 (100) |
| 192,000 | 16 (60) |

### 7.2.2. EX-FLASHER

Ex-Flasher is a vacuum bottom resid having a softening point of 21-32°C (70-90°F). The characteristics of the crude, its specific gravity, API gravity (°API), paraffin content (% by weight), aromatic content (% by weight), asphaltene content (% by weight) and viscosity (in centipoise) versus temperature profile, were determined experimentally and are summarized in Table VIII. The paraffin, aromatic, sulfur and asphaltene content were determined by the methods described in Section 7.2.3.

**TABLE VIII**

| EX-FLASHER CHARACTERISTICS | |
|---|---|
| Specific Gravity | = 1 |
| API Gravity (calculated | = 9.3°API |
| Paraffin content | = 24.9% (w/w) |
| Aromatic content | = 64.6% (w/w) |
| Asphaltene content | = 10.5% (w/w) |
| Sulfur content | = 3.4% (w/w) |

| Viscosity (CPS) | Temp. °C (°F) |
|---|---|
| 64,000 | 48 (118) |
| 33,000 | 53 (128) |
| 20,000 | 59 (138) |
| 14,000 | 64 (148) |
| 9,000 | 70 (158) |
| 4,100 | 76 (168) |
| 2,000 | 82 (179) |
| 1,800 | 87 (189) |
| 950 | 91 (196) |
| 900 | 93 (199) |
| 640 | 99 (211) |
| 500 | 104 (220) |

### 7.2.3. METHODS FOR DETERMINING HYDROCARBON CHARACTERISTICS, INCLUDING ASPHALTENE CONTENT

Viscosity versus temperature profiles were obtained by heating the oils to temperatures given in the tables VII-XIII and measuring viscosities in a Rheomat 30 rheometer (Contraves AG), at an approximate shear rate of 30 sec.⁻¹.

The paraffin, asphaltene and aromatic contents of the sample hydrocarbons were obtained by a method in which the hydrocarbons are dispersed in n-heptane, the asphaltenes removed by filtration and the remaining components separated based on their solubilities in n-heptane and methylene chloride. The asphaltene fraction (the precipitate) is filtered from a dispersion of the hydrocarbon in n-heptane. The paraffin fraction is that portion soluble in n-heptane. The aromatic fraction is that portion soluble in methylene chloride, but not in n-heptane.

The materials used are as follows: an analytical balance, accurate to 0.1 milligram (mg), a blender (Osterizer Galaxy 14) and blades fitted to a 500 ml Mason jar, preweighed Whatman #1 paper, filter funnel, rotary evaporation apparatus, a 500 millimeter (mm) burette-type chromatography column, tared collection flasks, reagent grade methylene chloride, n-heptane (99 mole percent) and alumina adsorbent. The alumina was activated by heating it in an oven at 310°C for 12-14 hours. The alumina was cooled in a dessicator and stored in a tightly capped bottle prior to use. Chromatography columns packed 3/4 full were used.

Hydrocarbon samples of 1-2 g were quantitatively added to Mason jars containing 100 ml of n-heptane. After blending for 1-2 minutes at maximum speed, the jar and its contents were washed with an additional 100 ml of n-heptane. The dispersed sample was filtered through Whatman #1 paper and the filtrate colected into Erlenmeyer flasks. After introduction of the filtrate to the column, the effluent was collected into a tared evaporation flask. When n-heptane was completely eluted, 200 ml of methylene chloride was added to the column and the eluted material collected into another tared evaporation flask until the column ran dry.

The eluting solvents were removed using a rotating vacuum evaporator at temperatures appropriate to the solvents.

The tared filter paper and flasks were reweighed and the percentage of asphaltenes, paraffins, and aromatics were calculated based on the original weight of the sample. Individual samples were run in duplicate. All percentages apearing in the foregoing tables for paraffinic, aromatic and asphaltene content have been adjusted to 100% recovery for comparative purposes.

Sulfur content was assayed by a quantitative assay on a Leco sulfur analyzer.

### 7.2.4. PREATOMIZED FUELS

The US-A-4,618,348, presented examples detailing procedures for forming preatomized fuels and the properties of the resultant preatomized fuels.

### 7.3. OXIDIZED SULFUR COMPOUND REDUCTION EXPERIMENTS

### 7.3.1. FURNACE ASSEMBLY AND INSTRUMENTATION

The SOX reduction combustion tests were run in a Cleaver-Brooks 15 MM Btu/hr fire tube hot water boiler furnace equipped with instrumentation for operating condition monitoring. Access to the fire chamber is also provided for radiation and temperature measurements.

The furnace fuel intake line is equiped with a Micro-Motion model C50 mass flow meter which can accurately measure fuel flow independent of viscosity. Just downstream of this meter, instrumentation which monitors fuel temperature and pressure is present, providing a continuous record of these parameters during operation.

Furnace exhaust gases are continuously monitored using a Perkin-Elmer Multiple Gas Analyzer (MGA) model 1200, a mass spectrometer which continuously samples and monitors the exhaust for N₂, O₂, SO₂, H₂O, and CO₂. The assembly is also equipped with instrumentation which can monitor CO, NOX, and particulates within the exhaust gases.

The same boiler load (heat output of the boiler relative to its maximum rated capacity) or fuel input (on a Btu basis) was used for each series of tests. All other boiler conditions were maintained as stable as possible during each test . The design of the Cleaver-Brooks boiler system is such that the atomization air flow is relatively constant for all firing rates. Therefore, the atomizing air/fuel ratio will decrease as the fuel is increased, resulting in richer fuel/air mixtures being burned, and the air/fuel ratio will increase as the fuel is decreased, resulting in leaner fuel/air (excess O₂) mixtures being burned.

### 7.3.2. DETERMINATION OF SO₂ REMOVAL EFFICIENCY

Sulfur dioxide SO₂ removal efficiency is determined by measuring the baseline SO₂ concentration from produced by fuel being examined using the Perkin-Elmer Multiple Gas Analyzer. Comparisons were then made with the SO₂ emissions observed during combustion the fuel containing various sulfur sorbents. For these comparisons, all SO₂ concentrations were corrected to the "equivalent" concentration which would be observed if the excess O₂ in the burner was 3%, using the following conversion:
where [SO₂] is the observed SO₂ concentration and [O₂] is the excess concentration of oxygen (i.e. that above the ambient air concentration), both in volume precent.

In this way, the effect of varying O₂ concentration is negated, and the results of the separate experimental series can be directly compared.

The percent of SO₂ reduction observed when a sorbent additive is present, called % removal, is calculated by the following formula:
where [SO₂] is the observed SO₂ concentration for each fuel or fuel/sorbent mixture at each condition examined.

The removal efficiency (%RE) is determined by calculating the ratio of the (observed) % removal/the theoretical sulfur binding capacity of the sorbent (assuming it reacted stoichiometrically) and dividing this number by the % sulfur in the fuel, i.e.:
For example, if 30% sulfur dioxide removal was observed, the fuel contained 3.33% sulfur and amount of sorbent added could theoretically remove 2% of this sulfur, then:

### 7.3.3. PROFILE OF TEST PREATOMIZED FUEL

Ex-Flasher (see section 7.2.2. supra) was tested as preatomized fuel having a 70/30 hydrocarbon to water ratio. The aqueous phase contains 0.125% of Kelco K1A112 biopolymer and a surfactant package, is present at a level of 1/250 parts oil. The surfactant package is comprised of the following:

| Material | % |
|---|---|
| Pluronic F-38 | 47.24 |
| Tergitol NP-40 | 21.38 |
| Iconol DNP-150 | 21.38 |
| Basified Indulin AT | 10.00 |

Once the preatomized fuel is prepared, 500 ppm (to the aqueous phase) formaldehyde is added to prevent microbial degradation.

In triplicate combustion experiments, the following parameters were found:

**TABLE IX**

| Fuel | % Sulfur¹ | | % SO₂ at 3% O₂² | |
|---|---|---|---|---|
| | Analysis | Theoretical | Actual | Analysis |
| EX-FLASHER | 3.40 | 3.64 | 1937 | 1811 |
| EX-FLASHER | 3.40 | 3.70 | 1971 | 1811 |
| EX-FLASHER | 3.40 | 3.36 | 1791 | 1811 |

| | | | | |
|---|---|---|---|---|
| ¹The "analysis" % was measured by a quantitative S-assay prior to combustion; the "theoretical" % was calculated from the measured SO₂ observed during combustion. | | | | |
| ²The actual % was measured by the MGA during combustion; the "analysis" % is calculated based on the % S obtained in the analysis assuming 100% conversion to SO₂. | | | | |

### 7.3.4. USE OF LIMESTONE AS A SORBENT

Limestone, CaCO₃ (Pfizer, Inc. Marblewhite 325, a natural source fire-grind limestone), was added to the fuel in two concentrations, which if reacted stoichiometrically with the sulfur, would have reduced the sulfur in the fuel 1 and 2 percent respectively. The results of the SO₂ measurement observed during the furnace combustion are presented in Table X.

**Table X**

| Results of Limestone Sorbent Tests | | | | | | | |
|---|---|---|---|---|---|---|---|
| FUEL | SORBENT | AMOUNT | EXCESS 02 | BOILER LOAD | SO2(3%O₂) | % REMOV | %R EFF |
| EX-FLASHER | CaCO₃ | 1 | 3.2 | 49 | 1804 | 5 | 16 |
| | | 1 | 3.8 | 49 | 1744 | 8 | 26 |
| | | 1 | 5.7 | 49 | 1744 | 8 | 26 |
| | | 1 | 1.0 | 27 | 1839 | 3 | 9 |
| | | 1 | 2.1 | 27 | 1818 | 4 | 13 |
| | | 1 | 8.9 | 28 | 1749 | 8 | 26 |
| EX-FLASHER | CaCO₃ | 2 | 1.0 | 51 | 1805 | 5 | 8 |
| | | 2 | 2.3 | 51 | 1760 | 7 | 11 |
| | | 2 | 3.5 | 51 | 1724 | 9 | 14 |
| | | 2 | 5.8 | 51 | 1710 | 10 | 16 |
| | | 2 | 2.1 | 28 | 1776 | 6 | 9 |
| | | 2 | 2.9 | 28 | 1745 | 8 | 13 |
| | | 2 | 3.9 | 29 | 1722 | 9 | 14 |
| | | 2 | 4.4 | 28 | 1706 | 10 | 16 |
| | | 2 | 5.9 | 27 | 1668 | 12 | 19 |

As shown, the removal efficiency was higher with the lower amount of CaCO₃. Also, the reaction of sorbent with sulfur dioxide is dependent on the temperature profile (load) in the furnace, being more efficient at lower loads. This is not unexpected since, as temperature increases, the surfaces of the sorbents may fuse, reducing the available surface at which the SOX absorbing reactions can occur. The effects of these parameters are graphically presented in Figure 1.

### 7.3.5. USE OF LIMESTONE/SODA ASH ADMIXTURES AS SORBENTS

This series of experiments examined the effect of using limestone (CaCO₃)/soda ash (Na₂CO₃) admixtures as sulfur sorbents. The soda ash was mixed with the limestone at 3 levels, 1, 3, and 10% by weight. The results are presented in Table XI and, also, graphically presented in Figure 2.

The results, compared at three percent oxygen, show a significant improvement in removal efficiency as the percent of sodium carbonate is increased. A comparison of removal rates for the various sodium carbonate additions shows a moderate dependence on excess oxygen and no dependence on boiler load.

By subtracting the effects of the sodium carbonate, i.e., reducing the baseline sulfur dioxide level by the amount of sulfur the sodium carbonate would remove (assuming 100% of removal efficiency) interesting results were obtained, as shown in the final column. A marked improvement in removal efficiency as the percent Na₂CO₃ was increased. This is clearly a catalytic effect, since the absorbance due to the Na₂CO₃ was corrected for. Apparently, Na₂CO₃ exerts a synergestic effect on the absorbing capacity of the CaCO₃.

### 7.3.6. USE OF CALCIUM ACETATE AS A SORBENT

This series of experiments examined the effectiveness of calcium acetate (CaAc) as a sulfur sorbent. Since CaAc is water soluble, the "particle" size of the dissolved calcium sorbent is not dependent on the initial grinding. Thus, the effective particle size is quite small, and the material, therefore, a more effective sorbent.

The results of a series of tests confirmed this, the results for which are shown in Table XII.

**TABLE XII**

| Results of CaAc Sorbent Tests | | | | | | | |
|---|---|---|---|---|---|---|---|
| FUEL | SORBENT | AMOUNT | EXCESS O2 | BOILER LOAD | SO2(3%) | %REMOV | %R EFF |
| EX-FLASHER | CaAc | 2 | 2.2 | 49 | 1337 | 29 | 48 |
| | | 2 | 3.1 | 49 | 1326 | 30 | 49 |
| | | 2 | 4.0 | 48 | 1285 | 32 | 53 |
| | | 2 | 5.1 | 48 | 1263 | 33 | 54 |
| | CaAc | 2 | 2.2 | 28 | 1246 | 34 | 56 |
| | | 2 | 3.3 | 28 | 1210 | 36 | 59 |
| | | 2 | 4.2 | 28 | 1167 | 38 | 63 |
| | | 2 | 5.4 | 28 | 1125 | 40 | 66 |
| | | 2 | 5.9 | 28 | 1120 | 41 | 68 |

As shown, in tests performed at 30 and 50% loads, the CaAc sorbent demonstrated a 48-54% and a 56-68% removal efficiency, respectively.

### 7.3.7. USE OF LIMESTONE/CaAc MIXTURES AS SORBENTS

Because of the superior sorbent ability of CaAc observed in example 7.3.6., a series of experiments using limestone mixed with 10% CaAc was conducted. The results are presented in Table XIII, and graphically presented in Figure 3.

**TABLE XIII**

| Results of CaCO₃/CaAc Sorbent Tests | | | | | | | | |
|---|---|---|---|---|---|---|---|---|
| FUEL | SORBENT | AMOUNT | EXCESS O2 | BOILER LOAD | SO2(3%) | %REMOV | %R EFF | %RE-CaAc¹ |
| EX-FLASHER | CaCO3/10%CaAc | 2 | 1.4 | 51 | 1584 | 16 | 26 | 22 |
| | | 2 | 2.8 | 51 | 1561 | 18 | 29 | 24 |
| | | 2 | 4.1 | 51 | 1495 | 21 | 34 | 30 |
| | | 2 | 5.2 | 52 | 1429 | 24 | 39 | 36 |
| | | 2 | 5.4 | 51 | 1422 | 25 | 41 | 36 |
| | | 2 | 1.8 | 29 | 1534 | 19 | 31 | 26 |
| | | 2 | 3.0 | 29 | 1484 | 22 | 36 | 31 |
| | | 2 | 4.1 | 29 | 1409 | 25 | 41 | 38 |
| | | 2 | 5.2 | 29 | 1384 | 27 | 44 | 40 |

| | | | | | | | | |
|---|---|---|---|---|---|---|---|---|
| ¹ % Re-CaAc numbers provide the calcium utilization efficiency, assuming that all the CaAc present is utilized at 100% Stoichiometric efficiency. | | | | | | | | |

Although not quite as effective as the sodium carbonate, the SO2 removal efficiency of the limestone was doubled, even after correction for the CaAc, and assuming 100% efficiency for the CaAc (a very conservative assumption). This is significant since this sorbent combination will not have the problems with corrosion and/or fouling that might be experienced with the limestone/10% sodium carbonate combination.

It is apparent that many modifications and variations of this invention as hereinabove set forth may be made without departing from the scope thereof. The specific embodiments described are given by way of example only, and the invention is limited only by the terms of the appended claims.

## Claims

1. An improved method for reducing SOX emissions during combustion of a sulfur-containing combustible material wherein the improvement comprises adding to said combustible material, prior to combustion, 0.5-25% by weight of an admixture of 80-99.5% by weight insoluble sulfur sorbent and 0.5-20% by weight soluble sulfur sorbent, the solubility being based on water.

2. The method of claim 1 wherein the insoluble sulfur sorbent is an alkaline earth metal carbonate.

3. The method of claim 2 wherein the alkaline metal carbonate is selected from the group consisting of calcium carbonate, magnesium carbonate, and dolomite.

4. The method of claim 1 wherein the soluble sulfur sorbent is selected from the group consisting of sodium carbonate, sodium acetate, sodium formate, sodium propionate, calcium acetate, calcium formate, calcium propionate, magnesium acetate, magnesium formate, and magnesium propionate.

5. The method of at least one of claims 1 - 4 wherein the combustible material is selected from the group consisting of a sulfur-containing coal, a sulfur-containing coal-in-water slurry, a sulfur-containing hydrocarbon oil.

6. The method of at least one of claims 1 - 4 wherein the combustible material is a preatomized fuel formed from a sulfur-containing hydrocarbon.

7. The method of claim 6 comprises the precombustion steps of
a. emulsifying the hydrocarbon in water to form a preatomized fuel, and
b. adding to said preatomized fuel 0.5-25% by weight of said admixture of 80-99.5% by weight insoluble sulfur sorbent and the 0.5-20% by weight soluble sulfur sorbent.

8. The method of claim 7 wherein the sulfur-containing hydrocarbon is selected from the group consisting of a viscous crude oil, a viscous vacuum resid, a viscous visbreaker resid, a viscous catalytic hydrogenated resid, a viscous cutback tar, a viscous pyrolysis pitch, a viscous propane deasphalted tar, viscous ROSE bottoms, and a viscous Boscan Crude Oil.

9. A clean-buring fuel which produces low SOX emission when burned which comprises a sulfur-containing combustible material and 0.5-25% by weight admixture of 80-99.5% insoluble sulfur sorbent and 0.5-20% by weight soluble sulfur sorbent, the solubility being based on water.

10. The fuel of claim 9 wherein the insoluble sulfur sorbent is an alkaline earth metal carbonate.

11. The fuel of claim 10 wherein the alkaline earth metal carbonate is selected from the group consisting of calcium carbonate, magnesium carbonate and dolomite.

12. The fuel of claim 9 wherein the soluble sulfur sorbent is selected form the group consisting of sodium carbonate, sodium acetate, sodium formate, sodium propionate, calcium acetate, calcium formate, calcium propionate, magnesium acetate, magnesium formate, and magnesium propionate.

13. The fuel of at least one of claims 9 - 12 wherein the combustible material is selected from the group consisting of a sulfur-containing hydrocarbon oil and sulfur -containing coal-in-water slurry.

14. The fuel of claim 13 comprising a preatomized viscous sulfur-containing hydrocarbon.

15. The fuel of claim 14 wherein the sulfur-containing hydrocarbon is selected from the group consisting of a viscous crude oil, a viscous vacuum resid, a viscous visbreaker resid, a viscous catalytic hydrogenated resid, a viscous cutback tar, a viscous pyrolyses pitch, a viscous propane deasphalted tar, viscous ROSE bottoms, and a viscous Boscan Crude Oil.

16. A clean-burning fuel of claim 9 which comprises:
a. as sulfur-containing combustible material: 90 to 99% of a combustible preatomized fuel formed by emulsifying a vacuum bottom resid with water in a 70/30 ratio using 0.125% heteropolysaccharide biopolymer S-194 produced by Alcaligenes sp. ATCC 31961 and 1/250 parts oil of a surfactant package comprising 47.24% polyoxypropylene-polyoxyethylene block copolymer in prill form having a hydrophilic-lipophilic balance of 30.5, 21.38% nonylphenol polyethylene glycol ether having an average molecular weight of 1980 amu, 21.38% dinoylphenol ethoxylate having an average molecular weight of 6900 amu and 10% purified free acid pine lignin; and
b. 1 to 10% of the weight admixture comprising 90 to 99% CaCo₃ as insoluble sulfur sorbent and 1 to 10% Na₂Co₃ as soluble sulfur sorbent.

17. A clean-burning fuel of claim 9 which comprises:
a. as sulfur-containing combustible material: 90 to 99% of a combustible preatomized fuel formed by emulsifying a vacuum bottom resid with water in a 70/30 ratio using 0.125% heteropolysaccharide biopolymer S-194 produced by Alcaligenes sp. ATCC 31961 and 1/250 parts oil of a surfactant package comprising 47.24% polyoxypropylene-polyoxyethylene block copolymer in prill form having a hydrophilic-lipophilic balance of about 30.5, 21.38% nonylphenol polyethylene glycol ether having an average molecular weight of 1980 amu, 21.38% dinonylphenol ethoxylate having an average molecular weight of 6900 amu and 10% purified free acid pine lignin; and
b. 1 to 10% of the weight admixture comprising 90 to 99% CaCO₃ as insoluble sulfur sorbent and 1 to 10% calcium acetate as soluble sulfur sorbent.

## Patentansprüche

1. Ein verbessertes Verfahren zum Reduzieren von SOX Emissionen während einer Verbrennung eines schwefelhaltigen, brennbaren Materials, wobei die Verbesserung die Zugabe von 0.5 - 25 Gew.% einer Zumischung von 80 - 99.5 Gew.% unlöslichem Schwefel-Sorptionsmittel und 0.5 - 20 Gew.% löslichem Schwefel-Sorptionsmittel vor der Ver-brennung zu diesem brennbaren Material vorsieht, wobei die Löslichkeit auf Wasser bezogen ist.

2. Verfahren nach Anspruch 1, dadurch gekennzeichnet, daß das unlösliche Schwefel-Sorptionsmittel ein Carbonat eines alkalischen Erdmetalls ist.

3. Verfahren nach Anspruch 2, dadurch gekennzeichnet, daß das alkalische Metallcarbonat aus der Gruppe ausgewählt ist, die aus Calziumcarbonat, Magnesiumcarbonat und Dolomit besteht.

4. Verfahren nach Anspruch 1, dadurch gekennzeichnet, daß das lösliche Schwefel-Sorptionsmittel aus einer Gruppe ausgewählt ist, welche das Natriumcarbonat, Natriumazetat, Natriumformiat, Natriumpropionat, Calziumazetat, Calziumformiat, Calziumpropionat, Magnesiumazetat, Magnesiumformiat und Magnesiumpropionat umfaßt.

5. Verfahren nach wenigstens einem der Ansprüche 1 bis 4, dadurch gekennzeichnet, daß das brennbare Material aus einer Gruppe ausgewählt ist, welche eine schwefelhaltige Kohle, eine schwefelhaltige Kohle-in-Wasser-Aufschlämmung, ein schwefelhaltiges Kohlenwasserstofföl umfaßt.

6. Verfahren nach wenigstens einem der Ansprüche 1 bis 4, dadurch gekennzeichnet, daß das brennbare Material ein vorzerstäubter Brennstoff ist, der aus einem schwefelhaltigen Kohlenwasserstoff hergestellt ist.

7. Verfahren nach Anspruch 6, dadurch gekennzeichnet, daß vor der Verbrennung folgende Arbeitsschritt durchgeführt werden:
a. Emulgieren des Kohlenwasserstoffes in Wasser, um einen vorzerstäubten Brennstoff herzustellen und
b. Zugabe von 0.5 - 25 Gew.% der Zumischung aus 80 - 99.5 Gew.% unlöslichem Schwefel-Sorptionsmittel und 0.5 - 20 Gew.% löslichem Schwefel-Sorptionsmittel zu diesem vorzerstäubten Brennstoff.

8. Verfahren nach Anspruch 7, dadurch gekennzeichnet, daß der schwefelhaltige Kohlenwasserstoff aus einer Gruppe ausgewählt wird, welche ein viskoses Erdöl, einen viskosen Vakuumrückstand, einen viskosen Rückstand aus einer Visbreaker-Anlage, einen viskosen, katalytisch hydrierten Rückstand, einen viskosen Verschnitteer, einen viskosen Pyrolyseteerrückstand, einen viskosen propandeasphaltierten Teer, viskose ROSE Bodensätze und ein viskoses Boscan Erdöl umfaßt.

9. Ein sauber brennender Brennstoff, der beim Brennen eine geringe SOX-Emission erzeugt und der aus einem schwefelhaltigen brennbaren Material und 0.5 - 25 Gew.% Beimischung von 80 - 99.5 Gew.% unlöslichem Schwefel-Sorptionsmittel und 0.5 - 20 Gew.% löslichem Schwefel-Sorptionsmittel besteht, wobei die Löslichkeit auf Wasser bezogen ist.

10. Brennstoff nach Anspruch 9, dadurch gekennzeichnet, daß das unlösliche Schwefel-Sorptionsmittel ein Carbonat der Erdalkalimetalle ist.

11. Brennstoff nach Anspruch 10, dadurch gekennzeichnet, daß das Carbonat der Erdalkalimetalle aus der Gruppe ausgewählt ist, die aus Calziumcarbonat, Magnesiumcarbonat und Dolomit besteht.

12. Brennstoff nach Anspruch 9, dadurch gekennzeichnet, daß das lösliche Schwefel-Sorptionsmittel aus der Gruppe ausgewählt ist, die Natriumcarbonat, Natriumazetat, Natriumformiat, Natriumpropionat, Calziumazetat, Calziumformiat, Calziumpropionat, Magnesiumazetat, Magnesiumformiat und Magnesiumpropionat umfaßt.

13. Brennstoff nach wenigstens einem der Ansprüche 9 bis 12, dadurch gekennzeichnet, daß das brennbare Material aus der Gruppe ausgewählt ist, welche ein schwefelhaltiges Kohlenwasserstofföl und schwefelhaltige Kohle-in-Wasser-Aufschlämmung beinhaltet.

14. Brennstoff nach Anspruch 13, der einen vorzerstäubten, viskosen schwefelhaltigen Kohlenwasserstoff beinhaltet.

15. Brennstoff nach Anspruch 14, dadurch gekennzeichnet, daß der schwefelhaltige Kohlenwasserstoff aus der Gruppe ausgewählt ist, die ein viskoses Erdöl, einen viskosen Vakuumrückstand, einen viskosen Rückstand aus einer Visbreaker-Anlage, einen viskosen, katalytisch hydrierten Rückstand, einen viskosen Verschnitteer, einen viskosen Pyrolyseteerrückstand, einen viskosen, propandeasphaltierten Teer, viskose ROSE-Bodenrückstände und ein viskoses Boscan Erdöl umfaßt.

16. Ein sauber brennender Brennstoff nach Anspruch 9, der aus folgendem besteht:
a) als schwefelhaltiges brennbares Material: 90 - 99% eines brennbaren vorzerstäubten Brennstoffes, der durch Emulgieren eines Vakuum-Bodenrückstand mit Wasser in einem Verhältnis 70/30 hergestellt wurde, wobei 0,125% eines heteropolysacchariden Biopoymers S-194, hergestellt durch Alcaligenes sp. ATCC 31961 und 1/250stel Teil Öl einer grenzflächenaktiven Einheit aus 47.24% Polyoxypropylen-Polyoxyethylen-Block-Copolymer in granulierter Form, welches ein hydrophilisches-lipophilisches Gleichgewicht von 30.5 aufweist, 21.38% Nonylphenol-Polyethylen-Glycoläther, der ein durchschnittliches Molekulargewicht von 1980 amu hat, 21.38% Dinonylphenolethoxylat, welches ein durchschnittliches Molekulargewicht von 6.900 amu hat, und 10% gereinigtes, säurefreies Kiefernlignin benutzt wird; und
b. 1 - 10 Gew.% Beimischung, welche aus 90 - 99% CaCO₃ als unlösliches Schwefel-Sorptionsmittel und 1 - 10% Na₂CO₃ als lösliches Schwefel-Sorptionsmittel besteht.

17. Ein sauber brennender Brennstoff nach Anspruch 9, welcher aus folgendem besteht:
a. als schwefelhaltiges brennbares Material: 90 - 99% eines brennbaren, vorzerstäubten Brennstoffes, der durch Emulgieren eines Vakuum-Bodenrückstand mit Wasser in einem Verhältnis von 70/30 hergestellt wird, wobei 0.125% eines heteropolysacchariden Biopolymers S-194, hergestellt durch Alcaligenes sp. ATCC 31961 und 1/250stel Teil Öl einer grenzflächenaktiven Einheit aus 47.24% Polyoxypropylen-Polyoxyethylen-Block-Copolymers in granulierter Form, das ein hydrophilisches-lipophilisches Gleichgewicht von ungefähr 30.5 aufweist, 21.38% Nonylphenol-Polyethylen-Glycoläther, der ein durchschnittliches Molekulargewicht von 1980 amu aufweist, 21.38% Dinonylphenolethoxylat, welches ein durchschnittliches Molekulargewicht von 6.900 amu aufweist, und 10 % gereinigtes, säurefreies Kiefernlignin; und
b. 1 bis 10 Gew.% Beimischung , die 90 - 99% CaCO₃ als Schwefel-Sorptionsmittel und 1 bis 10% Calziumazetat als lösliches Schwefel-Sorptionsmittel aufweist.

## Revendications

1. Méthode améliorée de réduction des émissions de SOX pendant la combustion d'un matériau combustible contenant du soufre, caractérisée en ce que l'amélioration comprend le fait d'ajouter au dit matériau combustible, préalablement à la combustion, de 0,5 à 25 % en poids d'un mélange de 80 à 99,5 % en poids d'un adsorbant du soufre, insoluble, et de 0,5 à 20 % en poids d'adsorbant du soufre soluble, la solubilité étant basée sur l'eau.

2. Procédé selon la revendication 1, caractérisé en ce que l'adsorbant du soufre insoluble est un carbonate de métal alcalino-terreux.

3. Procédé selon la revendication 2, caractérisé en ce que le carbonate de métal alcalin est choisi dans le groupe qui consiste en le carbonate de calcium, le carbonate de magnésium et la dolomite.

4. Procédé selon la revendication 1, caractérisé en ce que l'adsorbant soluble du soufre est choisi dans le groupe qui consiste en le carbonate de sodium, l'acétate de sodium, le formiate de sodium, le propionate de sodium, l'acétate de calcium, le formate de calcium, le propionate de calcium, l'acétate de magnésium, le formiate de magnésium et le propionate de magnésium.

5. Procédé selon au moins une des revendications 1 à 4, caractérisé en ce que le matériau combustible est choisi dans le groupe qui consiste en un charbon contenant du soufre, une boue de charbon dans l'eau contenant du soufre, une huile hydrocarbonée contenant du soufre.

6. Procédé selon au moins une des revendications 1 à 4, caractérisé en ce que le matériau combustible est du fuel, pré-atomisé, formé à partir d'un hydrocarbure contenant du soufre.

7. Procédé selon la revendication 6 qui comprend les étapes de précombustion suivantes :
a) émulsion de l'hydrocarbure dans l'eau pour former un fuel pré-atomisé et
b) addition au dit fuel pré-atomisé de 0,5 à 25 % en poids du dit mélange de 80-99,5 % en poids d'adsorbant du soufre insoluble et de 0,5 à 20 % en poids d'adsorbant du soufre soluble.

8. Procédé selon la revendication 7, caractérisé en ce que l'hydrocarbure contenant du soufre est choisi dans le groupe formé d'une huile brute visqueuse, un résidu sous vide visqueux, un résidu visqueux de viscoréducteur, un résidu d'hydrogénation catalytique visqueux, un bitume fluxé visqueux, un brai de pyrolyse visqueux, un goudron désasphalté de propane visqueux, un fond de creuset de ROSE visqueux et une huile brute de Boscan visqueuse.

9. Fuel brûlant sans résidu de combustible qui produit une faible émission de SOX quand il brûle, qui comprenant un matériau combustible contenant du soufre et de 0 à 25 % en poids d'un mélange de 80-99,5 % d'adsorbant du soufre insoluble et de 0,5-20 % en poids d'adsorbant du soufre soluble, la solubilité étant basée sur l'eau.

10. Fuel selon la revendication 9, caractérisé en ce que l'adsorbant du soufre insoluble est un carbonate de métal alcalino-terreux.

11. Fuel selon la revendication 10, caractérisé en ce que le carbonate de métal alcalino-terreux est choisi dans le groupe formé du carbonate de calcium, du carbonate de magnésium et de la dolomite.

12. Fuel selon la revendication 9, caractérisé en ce que l'adsorbant de soufre, soluble, est choisi dans le groupe qui est formé par le carbonate de sodium, l'acétate de sodium, le formiate de sodium, le propionate de sodium, l'acétate de calcium, le formiate de calcium, le propionate de calcium, l'acétate de magnésium, le formiate de magnésium et le propionate de magnésium.

13. Fuel selon au moins une des revendications 9 à 12, caractérisé en ce que le matériau combustible est choisi dans le groupe formé d'une huile hydrocarbonée contenant du soufre et d'une boue de charbon dans l'eau contenant du soufre.

14. Fuel selon la revendication 13, qui comprend un hydrocarbure contenant du soufre, visqueux, préatomisé.

15. Fuel selon la revendication 14, caractérisé en ce que l'hydrocarbure contenant du soufre est choisi dans le groupe consistant en une huile brute visqueuse, un résidu sous vide visqueux, un résidu visqueux de viscoréduction, un résidu d'hydrogénation catalytique, visqueux, un bitume fluxé visqueux, un brai de pyrolyse visqueux, un bitume fluxé de propane, visqueux, un fond de creuset de ROSE visqueux et une huile brute Boscan visqueuse.

16. Fuel brulant sans résidu de combustible selon la revendication 9, qui comprend :
a) comme matériau contenant du soufre : 90 à 99 % d'un fuel pré-atomisé combustible obtenu par mise en émulsion d'un résidu de fond de cuve sous vide avec de l'eau dans le rapport 70/30 en utilisant 0,125 % du biopolymère S-194 hétéropolysaccharidique, produit par Alcaligènes sp. ATCC 31961 et 1/250 parties d'huile d'une combinaison de tensioactifs comprenant 47,24 % d'un copolymère bloc polyoxypropylène/polyoxyéthylène sous forme de granulés ayant un bilan hydrophile/lipophile de 30,5, 21,38 % d'un éther de nonylphénol et de polyéthylène glycol ayant un poids moléculaire moyen de 1980 amu, 21,38 % d'éthoxylate de dinonylphénol ayant un poids moléculaire moyen de 6900 amu et 10 % de lignine de pin purifiée exempte d'acide, et
b) 1 à 10 % du poids de mélange comprenant de 90 à 99 % de Co₃Ca comme adsorbant du soufre insoluble et de 1 à 10 % de Co₃Na₂ comme adsorbant du soufre soluble.

17. Fuel brulant sans résidu de combustible selon la revendication 9, qui comprend :
a) comme matériau combustible contenant du soufre : de 90 à 99 % d'un fuel combustible pré-atomisé produit par mise en émulsion d'un 〈〈 résidu 〉〉 de fond de cuve sous vide avec de l'eau dans un rapport 70/30 en utilisant 0,125 % des biopolymères hétéropolysaccharidiques S-194 produits par Alcaligènes sp. ATCC 31961 et 1/250 parties d'huile d'une combinaison d'agents tensioactifs comprenant 47,24 % de copolymère bloc polyoxypropylène-polyoxyéthylène sous forme de granulés ayant un bilan hydrophile/lipophile d'environ 30,5, 21,38 % d'éther de nonylphénol et de polyéthylèneglycol ayant un poids moléculaire moyen de 1980 amu, 21,38 % d'éthoxylate de dinonylphénol ayant un poids moléculaire moyen de 6900 amu, et 10 % de lignine de pin purifiée exempte d'acide, et
b) 1 à 10 % du poids du mélange comprenant de 90 à 99 % de Co₃Ca comme adsorbant du soufre insoluble et de 1 à 10 % d'acétate de calcium comme adsorbant du soufre soluble.
